

M. A. ADAM,  
TREATMENT OF CELLULOSE OR MATERIALS CONTAINING CELLULOSE,  
APPLICATION FILED MAR. 9, 1920.

1,402,201.

Patented Jan. 3, 1922.



Inventor:

Matthew Atkinson Adams,  
By Bynnes, Townsend &  
Brickington, Attorneys.

# UNITED STATES PATENT OFFICE.

MATTHEW ATKINSON ADAM, OF LONDON, ENGLAND.

## TREATMENT OF CELLULOSE OR MATERIALS CONTAINING CELLULOSE.

1,402,201.

Specification of Letters Patent.

Patented Jan. 3, 1922.

Continuation of application Serial No. 798,451, filed October 31, 1913. This application filed March 9, 1920. Serial No. 364,366.

To all whom it may concern:

Be it known that I, MATTHEW ATKINSON ADAM, a subject of the King of Great Britain and Ireland, residing at London, England, 5 have invented certain new and useful Improvements in and Relating to the Treatment of Cellulose or Materials Containing Cellulose, of which the following is a specification.

10 This invention relates to improvements in processes for the chemical treatment of cellulosic materials such as wood, which have for their object either the obtaining of more or less pure cellulose or by action upon the 15 cellulose or other components to produce sugar or other valuable products, and combinations of such processes.

As the result of experiment, I have ascertained that if, in such processes, the degree 20 of sub-division of the solid woody material treated, the amount of liquid matter admixed therewith, or the mechanical treatment of the mixture, or more than one of these factors be adjusted to secure during the 25 treatment that the mass be in the condition of a pulp or more or less fluid suspension, the advantages obtained in acceleration of the reaction or in other directions, or both, more than overcome the additional cost involved in bringing about the changed condition.

In particular, the result is to render continuously operating apparatus, with their advantages of high capacity, saving in capital outlay, labor and fuel, available for use 35 in such processes.

Thus I have found that by heating ground wood with bisulphite lye of standard composition to a temperature of 170° C., the 40 pulpy mass containing say 90% of water, the material was converted into chemical pulp in some 30 minutes, it being then apparently free from all incrusting matter and being more or less pure cellulose. This 45 result is only obtainable under these conditions of temperature in present practice in some 20 hours.

Again I have succeeded in obtaining from 50 sawdust ground to a pulp with water, mixed with a small quantity of acid and heated under pressure, the same amount of sugar as was obtainable where according to the latest proposals the acid is mixed with the sawdust in the presence of a minimum of 55 moisture and similarly heated, and in the

former case there were produced far smaller quantities of secondary products which, as is known, are a source of great trouble in attempts to ferment the sugar.

According to the present invention therefore in the treatment of woody cellulosic materials for purposes as indicated, the materials are before subjection to digestion brought to the condition of a fluent or mobile pulp and then preferably treated in apparatus adapted for continuous ingress and egress of the pulp, and, if desired, regeneration of heat between the treated material and that awaiting treatment.

The accompanying drawing shows diagrammatically how the treatment of waste wood may be carried out in one form and in continuous apparatus according to the present invention.

The material is transported from the heap, 1, by a conveyor, 2, to a pulverizer, 3, which may be an emery or other mill, into which it is introduced with an appropriate amount of extremely dilute acid supplied from a tank, 4, through a pipe, 5. This supply of liquid is regulated so as to yield a pulp containing say 90 to 92% of water and in which the amount of acid, e. g., hydrochloric, sulphuric or sulphurous acids, is present to the extent of some 0.5 to 2 parts by weight 85 to 100 parts by weight of dry wood. The pulped mass enters the pulp pit, 6, from which it is withdrawn by the feed pump, 7, and forced into the heater or digester. This includes a pipe, 8, having a pressure equalizer, 9, the pulp flowing along the pipe, 8, to the further extremity which is enclosed in the steam jacket, 9<sup>a</sup>, and returning by the bend, 10, to a jacket, 11, surrounding a portion of the pipe, 8, the mass during its flow 90 through the jacket imparting some of the heat it acquired when passing through the jacket, 9<sup>a</sup>, to material flowing through the pipe 8. The pulp leaves the jacket, 11, by the pipe, 12, and is now ready to be freed of 95 its liquid matter, the length of tube 8 enclosed in the jacket, 9<sup>a</sup>, and the velocity of flow of the pulp having been so chosen that the pulp has been maintained for a sufficient time, at the predetermined temperature, say, 105 150° C., and the transfer of heat in the jacket, 11, having been such as to cool the material to a convenient temperature for filtration say, to 80° to 95° C.

It will be understood that if the resistance 110

in the pipes from the heating region to the point of exit is insufficient to avoid ejection of the material a reducing valve or other suitable device, 13, may be introduced in the pipe 12.

The solid matter may now be separated from the liquid in a variety of ways, especially as the pressure required is relatively low and the necessary time short. It is best 10 however where a certain degree of pressure is to be employed to apply this gradually rather than to apply a heavy load at first.

In the drawing this separation is shown as effected in two stages. The material first 15 passes onto an endless web 14 having a suction box 15 as is used in drying wood pulp. During the passage of the material upon this web, which may occupy 2 to 3 minutes or thereabouts, the liquid is drawn away by 20 the wet air pump 16, as also any washings to which the mass may be subjected.

The more or less solid mass 17 is now borne from the web 14 by rollers 18 to a press composed of endless bands 19 and 19' 25 gradually approaching each other and thus gradually exerting increased pressure upon the material, the material being finally discharged at 20 after subjection during say for 2 to 5 minutes to a pressure rising to 30 say 100 lbs. per square inch. It then contains about 50% or but little more of moisture, is fairly strong and can be gasified in a gas producer 22 to which it is fed by a conveyer, 21, to yield fuel for steam and 35 power raising for the process.

The liquid matters from the pump 16 and the collecting tray 23 of the band press are passed by the pipe 24 to a pump 25 by which, as the liquid is still practically at 40 the temperature at which it left the pipe 12, it is passed through the jacket 26 in order still further to save heat by transfer to the pulp flowing through the pipe 8. The more or less completely cooled liquid now leaves 45 the system at 27 and is then treated in the known way for the recovery of its valuable constituents.

The process may of course be carried out in other suitable forms of apparatus. Apparatus which is well-suited to the purpose 50 is shown in the patent to Testrup & Rigby 1,160,464 of November 16, 1915.

When applying the invention in this aspect to the manufacture of chemical wood pulp, the barked and trimmed logs can be ground wet in the way usual in making mechanical pulp, and preferably by the hot grinding process, when after separation of a suitable portion of the excess of water a 60 concentrated bisulphite or other digestive agent may be added to the material and the procedure described in connection with preceding example be adopted, the particular means employed for eventually separating

the pulp and lye being such as experience 65 directs. On the other hand, the wood may be ground directly into the digestive agent with advantage.

By carrying out processes of the chemical treatment of woody cellulosic bodies on lines 70 such as indicated, control of the rapidity, degree and course of the reaction becomes possible, and it is for example possible where the recovery of products from the liquors is sought, to minimize the formation 75 of deleterious secondary products by using a lower working temperature and a corresponding greater superincumbent pressure in the digesters. Where continuous appliances are used the excess pressure can for 80 example be attained by mechanically or chemically giving artificial viscosity or pastiness to the pulp and so increasing the pressure necessary to force the matter into 85 and from the apparatus.

Where the material is ground in order to produce the pulp it may in certain circumstances be more advantageous to grind it dry instead of wet as above described, particularly where no regard is paid to the fibre 90 length of the resulting end product or the product is required as wood meal or for like purpose. The dry grinding gives a product of extreme fineness and one therefore especially susceptible to rapid action. It may 95 be convenient where the raw product, e. g., waste wood, sawdust, is of mixed character to screen it, and to treat in separate units the portion composed of fine particles, this giving rapidly the desired result and yielding the fuel material for the process, while the coarse material yields after treatment 100 material of sufficiently long fibre to be available for paper making.

It is important to observe that apart from 105 moisture content and degree of subdivision of the material, mechanical beating or pulping can be brought to play a large part in the production of the pulp and in particular in the homogenizing of the material.

It should be observed that when employing 110 apparatus through which the material continuously flows as described all the advantages of quick heating and cooling are obtained without however the walls of the digester varying in temperature so that at all points during working the temperature 115 remains practically invariable, and lead or other linings can be safely employed without fear of rupture or buckling.

By the expression "in a finely subdivided form" in the appended claims, it is to be understood that the same refers to material which is pulverized or of such fineness that it is capable upon intimate mixing with water of forming a true pulp, which will flow 125 freely. It will be readily understood that this condition is not practically attainable

with the use of cellulosic materials which are coarser in their nature than relatively fine sawdust.

This application is a continuation of my 5 prior application Serial No. 798,451, filed October 31, 1913, and is filed in substitution thereof.

I claim:

1. In a process of treating woody matter 10 in a finely subdivided form, the steps which consist in forming thereof a fluent pulp with an added chemical solution, and then subjecting the said pulp in a continuous stream of digestion under heat and pressure.

15 2. In the process of treating cellulosic materials, the steps which consist in commingling the cellulosic materials in finely subdivided form with sufficient water to form therewith a fluent pulp and with a chemical 20 digestive agent, subsequently passing the said pulp continuously through a suitable digester while maintaining therein sufficient heat and pressure to accomplish the desired digestion, and passing the pulp directly 25 from the digester to heat regenerating means.

3. In the process of hydrolyzing cellulosic materials, the steps which consist in commingling the cellulosic material in subdivided form 30 with sufficient water to form therewith a fluent pulp and with a hydrolyzing agent, and subsequently passing the said pulp continuously through a suitable digester while maintaining therein sufficient heat 35 and pressure to accomplish the desired hydrolysis.

4. In a process of making sugar from cellulose, the steps which consist in commingling cellulosic material in subdivided form 40 with sufficient water to form therewith a fluent pulp and with an acid hydrolyzing agent, and subsequently passing the said pulp continuously through a suitable digester while maintaining therein sufficient heat 45 and pressure to accomplish the desired hydrolysis.

5. A method of hydrolyzing wood consisting in grinding the same to a fine condition of subdivision to produce a pulp with 50 a hydrolyzing liquid with which it is admixed, the pulp then with all of its water being continuously forced through heating and heat regenerating elements and the liquid

matter being then separated from the solid 55 matter; at set forth.

6. A method of treating woody cellulosic materials comprising reduction to pulp with an added chemical digestive agent heating the pulp under pressure, forcing the 60 treated pulp with all its water through heating and heat regenerating elements, thereby cooling the same to a temperature suitable for filtration, separating the liquid matter from the solid matter and recovering the 65 heat of the separated liquid matter by means of heat regenerating elements.

7. A method of treating woody cellulosic materials comprising reduction to pulp with an added chemical digestive agent heating 70 the pulp under pressure, forcing the treated pulp through heating and heat regenerating elements, thereby cooling the same to a temperature suitable for filtration, separating the liquid matter from the solid matter, recovering the heat from the separated liquid matter by means of heat regenerating elements and utilizing the solid matter for the 75 production of heat for the heating elements.

8. A method for the economic manufacture of sugar from woody cellulosic materials comprising the reduction to pulp with an added acid, subjecting the pulp to heat and pressure, separating the liquid matter from the solid matter, recovering heat from 85 the separated liquid matter and utilizing the solid matter for the production of heat in the process.

9. The method herein described of treating wood, consisting in grinding the wood 90 while subjected to an acid solution to form a pulp, heating the pulp to digest the same, removing a portion of the liquid, subjecting the mass to pressure, and then delivering the solid material to a gas producer. 95

10. The method herein described of treating wood, consisting in grinding the wood while subjected to an acid solution to form a pulp, subjecting the pulp to the action of heat to digest the pulp, removing a portion 100 of the liquid, subjecting the mass to pressure, delivering the solid material to a gas producer, and utilizing the extracted liquid to assist in heating the pulp.

In testimony whereof I affix my signature. 105

MATTHEW ATKINSON ADAM.